

3,295,980

**INCREASED EFFICIENCY WITH MUCOCHLORIC ACID HARDENING BY USE OF 4-SUBSTITUTED URAZOLES**

William W. Rees and William H. Russell, Rochester, N.Y., assignors to Eastman Kodak Company, Rochester, N.Y., a corporation of New Jersey  
 No Drawing. Filed Dec. 21, 1964, Ser. No. 420,196  
 6 Claims. (Cl. 96—109)

This invention relates to photographic elements, more particularly photographic silver halide emulsions containing fog-inhibiting agents and hardeners.

For most photographic applications adequate levels of hardness for the gelatin-silver halide photographic emulsion must be maintained. Ordinarily, photographic emulsions on storage tend to lose sensitivity and become fogged, i.e., developable without exposure to light. Therefore, it is desirable in such emulsions to have present substances which act as fog inhibitors and stabilizers therein. In the processing of photographic emulsions, it is important that the emulsion layer maintain satisfactory physical strength so as to resist physical and environmental degradation. Urazole has been considered a very satisfactory additive to photographic emulsions to exert a stabilizing and fog-inhibiting effect thereon. However, urazole as an antifogging agent has been restricted to use in conjunction with certain types of gelatin hardeners since it has the undesirable property of reacting with aldehyde-type gelatin hardeners, resulting in a detrimental effect on hardening by the aldehyde-type hardener.

One object of our invention is to provide photographic emulsions containing both stabilizer (antifogging) and aldehyde-type hardener which do not detract from each other's effectiveness in the emulsion. Another object of our invention is to provide photographic gelatin-silver halide photographic emulsions containing as the hardener, a halogen substituted aldehyde acid compound and, as the stabilizer, a compound of the urazole type therein. Other objects of our invention will appear herein.

We have found that by using as the aldehyde type gelatin hardener a halogen substituted aldehyde acid and by using as the antifogging or stabilizer a urazole substituted with an alkyl or aryl group or a hydrazide of maleic or phthalic acid both the stabilizing action and the hardening action of the respective compounds in the photographic emulsions are obtained with good effect.

The gelatin hardeners which have been found useful in our invention are those which have been described and claimed in U.S. Patent No. 2,080,019 of Frank L. White, particularly mucochloric acid or mucobromic acid. As a stabilizer or antifogging, compounds which have been found to be effective in the presence of mucochloric or mucobromic acid are substituted urazoles having the formula:



wherein R is either H, alkyl or aryl, only one of the R's being hydrogen. Also useful in this connection are the monoacyl or diacyl derivatives of compounds having this formula as for example the diacetyl derivative of 4-phenyl urazole. Compounds in accordance with this structural formula which are especially useful in this connection are 4-phenyl urazole, 1-phenyl urazole, 4-ethyl urazole, 4-naphthyl urazole and the like. Other compounds of this type which are useful in this connection are maleic acid hydrazide and phthalic acid hydrazide.

Typical alkyls which can be used as substituents are methyl, ethyl, propyl, butyl, etc. Typical aryls or aralkyls

which can be used as substituents are phenyl, tolyl, xylyl, naphthyl and the like including benzyl.

The hardening agent employed may be present in any amount which exhibits hardening action on the gelatin. As a rule the amount of halogen substituted aldehyde acid used will be within the range of 0.1–0.5%, based on the weight of the gelatin in the emulsion. The antifogging agents specified exert an antifogging effect in most any concentration. However, ordinarily the antifogging agent used in combination with the halogenated aldehyde acid compound in accordance with our invention will be present in an amount of .5–5%, based on the weight of the gelatin in the silver halide emulsion. Whereas when the urazole derivatives of our invention are utilized with other aldehyde hardeners there is ordinarily an effect on one by the other so as to interfere with their respective hardening (hardeners) or stabilizing (urazoles) actions, in the combination in accordance with the invention the hardening effectiveness and the stability effectiveness are maintained or in some cases increased when used in photographic emulsions.

The following examples illustrate more specifically the invention:

**EXAMPLE 1**

A coarse-grain gelatin-silver bromoiodide emulsion containing 139 grams gelatin per silver mole such as adapted for X-ray material was ripened to optimum sensitivity by adding the desired sensitizing agents and digesting. There was added thereto, as the hardener, 0.29 gram of mucochloric acid per gram molecular weight of silver (or per 139 grams of gelatin) in the emulsion plus addenda such as may be added in the making of photographic emulsions. In one sample of the emulsion no antifogging was used. To another sample, urazole was added and to three others were added, respectively, 4-phenyl urazole, 4-ethyl urazole and 4-naphthyl urazole. The emulsion samples were coated out onto cellulose triacetate base and the film samples thus obtained were tested for percent vertical swell of the gelatin emulsion layers in an aqueous bath having a pH of 10 and in distilled water each in relation to the dry layers. The melting points of each of the samples was also determined. The results obtained with the various samples were as follows:

Table I

| Addendum              | G./Ag<br>mole | Percent Vertical<br>Swell |                    | M.P.<br>(° F.) |
|-----------------------|---------------|---------------------------|--------------------|----------------|
|                       |               | pH 10.0<br>Buffer         | Distilled<br>Water |                |
| Control.....          | 0             | 459                       | 426                | >212           |
| Urazole.....          | 2.0           | 579                       | 647                | 95             |
| Phenyl urazole.....   | 2.0           | 369                       | 367                | >212           |
| Ethyl urazole.....    | 2.0           | 328                       | 361                | >212           |
| Naphthyl urazole..... | 2.0           | 380                       | 377                | >212           |

The percent vertical swell is obtained by determining the percentage of swelling of the various layers after they have been immersed for a short time in distilled water, or in water having a pH of 10 as the case may be, at 20° C. The melting point of the photographic emulsion layer is determined by placing the layer in water and slowly increasing the temperature thereof until the layer disintegrates from the support on which it has been coated.

**EXAMPLE 2**

In a similar procedure as in the preceding example several different aldehyde type hardeners were used, namely mucochloric acid, formaldehyde and succinaldehyde and the antifogging agent used was 4-phenyl urazole at a level of 2.0 grams per silver mole. The results obtained with and without the antifogging agent both as to percent ver-

tical swell in distilled water and as to the melting points of the photographic emulsion layers were as follows:

Table II

| Hardener, g./Ag mole  | 4-phenyl urazole | Percent Vertical Swell, Distilled Water | M. P. (° F.) |
|-----------------------|------------------|-----------------------------------------|--------------|
| Mucochloric acid 0.29 | —                | 422                                     | 197          |
| Mucochloric acid 0.29 | +                | 388                                     | 212          |
| Formaldehyde 0.20     | —                | 291                                     | 194          |
| Formaldehyde 0.20     | +                | 511                                     | 101          |
| Succinaldehyde 0.70   | —                | 656                                     | 94           |
| Succinaldehyde 0.70   | +                | 1,003                                   | 86           |

**EXAMPLE 3**

A coarse grain silver bromoiodide gelatin emulsion was chemically sensitized. The emulsion contained 139 grams of gelatin per mole of silver halide. There was added thereto 0.29 gram of mucochloric acid per mole of silver halide. The emulsion was divided into several portions and 1-phenyl urazole was added in the parts given. Each portion was then coated onto polyethylene terephthalate film support. A sample of each was exposed on an intensity scale sensitometer and processed for 6 minutes in Kodak Rapid X-ray Developer. The vertical swell, relative speed and melting point were determined. The following results were obtained:

| 1-Phenyl Urazole (g./mole<br>of silver halide) | Relative<br>Speed <sup>a</sup> | Percent<br>Vertical<br>Swell | Melting<br>Point<br>(° F.) |
|------------------------------------------------|--------------------------------|------------------------------|----------------------------|
| 0                                              | 100                            | 482                          | 206                        |
| 0.5                                            | 89                             | 474                          | 196                        |
| 1.0                                            | 87                             | 480                          | 196                        |
| 2.0                                            | 87                             | 509                          | 193                        |

**EXAMPLE 4**

A coarse grain silver bromoiodide gelatin emulsion as described in the preceding example was treated with the addenda described below and coated on polyethylene terephthalate film support. The amount of swell obtained was determined. It was found that the use of maleic hydrazide as the antifoggant resulted in substantially the same swelling characteristics as where the mucochloric acid hardener was used without antifoggant. The material added, proportions thereof and the swelling characteristics were as follows.

### Feature:

|                                          |     |
|------------------------------------------|-----|
| Percent swell<br>in developer<br>acid/Ag | 322 |
| m muco-                                  | 364 |
| ide + 0.29                               | 328 |

|   |                                                                             |     |
|---|-----------------------------------------------------------------------------|-----|
| 5 | Control + 0.75 gram urazole + 0.29 gram muco-chloric acid / Ag mole         | 364 |
|   | Control + 0.75 gram maleic hydrazide + 0.29 gram mucochloric acid / Ag mole | 328 |

The invention has been described in considerable detail with particular reference to certain preferred embodiments thereof, but it will be understood that variations and modifications can be effected within the spirit and scope of the invention as described hereinabove, and as defined in the appended claims.

15 as defined in  
We claim:

1. A light sensitive gelatin-silver halide emulsion containing as a hardener therein a halogen substituted aldehyde acid compound selected from the group consisting of mucochloric acid and mucobromic acid and as an anti-fogging agent therein a compound selected from the group consisting of the compounds having the following structural formula.



R being selected from the group consisting of H, alkyl, aryl, and aralkyl only one R being hydrogen, the mono-  
30 acetyl and diacetyl derivatives of these compounds, maleic acid hydrazide, and phthalic acid hydrazide.

2. A light sensitive gelatin-silver halide emulsion containing as a hardener therein mucochloric acid and as an antifoggant 4-phenyl urazole.

35 3. A light sensitive gelatin-silver halide emulsion containing as a hardener therein mucochloric acid and as an antifoggant 4-ethyl urazole.

4. A light sensitive gelatin-silver halide emulsion containing as a hardener therein mucochloric acid and as an antifoggant 4-naphthyl urazole.

40 5. A light sensitive gelatin-silver halide emulsion containing as a hardener therein mucochloric acid and as an antifoggant 1-phenyl urazole.

6. A light sensitive gelatin-silver halide emulsion containing as a hardener therein mucochloric acid and as an antifoggant maleic hydrazide.

45

No references cited.

50 NORMAN G. TORCHIN, *Primary Examiner.*  
J. H. RAUBITSCHEK, *Assistant Examiner.*